

Sept. 12, 1939.

H. L. REED

2,172,683

MINING PROCESS

Filed Aug. 10, 1937

3 Sheets-Sheet 1



FIG. 1.

Inventor  
Howard L. Reed.  
By J. Vincent Martin  
and  
Ralph R. Downing.  
Attorneys

Sept. 12, 1939.

H. L. REED

2,172,683

MINING PROCESS

Filed Aug. 10, 1937

3 Sheets-Sheet 2



Fig. 3.

Fig. 2. Inventor

Howard L. Reed.

By

J. Vincent Martin  
and  
Ralph R. Browning  
Attorneys

Sept. 12, 1939.

H. L. REED

2,172,683

MINING PROCESS

Filed Aug. 10, 1937

3 Sheets-Sheet 3



Fig. 4.

Inventor

Howard L. Reed.

J. Vincent Martin  
and  
Ralph R. Browning  
Attorneys

## UNITED STATES PATENT OFFICE

2,172,683

## MINING PROCESS

Howard L. Reed, Houston, Tex., assignor of eleven  
and one-third per cent to Fohs Oil Company

Application August 10, 1937, Serial No. 158,305

4 Claims. (Cl. 262—3)

This invention relates to a process of mining and more particularly has reference to the removal of minerals from a considerable distance below the surface of the ground without the difficulties previously attendant upon mining of such ores.

In the past, minerals have been removed from the ground in a number of ways, chief among which are the removal by simple excavation and bodily removal, and in some instances, by the circulation of a fluid medium for the purpose of bringing the minerals to the surface in the form of solutions. The present invention has reference to the latter general class of mining processes.

The mining of minerals by means of circulated fluids has in the past been limited to those minerals which could be melted or taken up by an aqueous displacement medium. The most noted process of removing a mineral by means of an aqueous medium is the well-known Frasch process, widely utilized in the mining of sulphur. In this process superheated water is forced into the sulphur well to the sulphur-bearing limestone beds, and by virtue of the stored heat in the water the sulphur is melted and caused to flow to the surface of the ground. However, the sulphur occurs in a relatively pure form in nature and is not changed chemically nor dissolved to any substantial degree during the process.

It is an object of this invention to provide a mining process by which minerals may be more cheaply and readily removed from the earth.

It is a further object to provide a process of mining which will enable the ready removal of minerals from hitherto inaccessible ore deposits.

It is an object of this invention to provide a mining process whereby mineral ores are not soluble in or meltable by an aqueous circulating medium may be removed from the ground.

It is a further object of this invention to provide a mining process by which mineral ores highly insoluble in a liquid medium in their natural state may be removed from the ground through the circulation of a liquid medium.

It is a further object of this invention to provide a mining process by which mineral ores normally extremely difficult to remove by any previously known process may be readily removed from the ground.

It is a further object of this invention to provide a mining process of the liquid displacement type which will have a broader application than previously known processes of this general nature using aqueous displacement media.

It is a further object of this invention to provide a mining process employing a liquid displacement medium and to provide a liquid displacement medium for such process which will eliminate many of the heat losses and other disadvantages inherent in previously employed circulating media.

It is a further object of this invention to provide a mining process for the removal of ores from the earth through the use of a circulating medium which will readily dissociate the various minerals from the gangue and remove them to the surface, and from which the various minerals may be readily extracted.

It is a further object of this invention to provide a circulating medium for use in removing mineral ores which circulating medium is not susceptible to the temperature limitations of a superheated aqueous medium which has a relatively high vapor pressure, but which may be readily vaporized to recover the minerals therefrom.

It is a further object of this invention to provide an improved process of mining, employing a liquid circulating medium and for removing the minerals from the circulating medium.

It is a further object to provide a liquid circulating medium for a process of mining, the chemical activity of which will increase with increase in temperature.

It is a further object to provide a liquid circulating medium for a process of mining, which medium will more readily than water or other aqueous medium take into solution the minerals to be removed.

It is the object of this invention to transform minerals and native metals to substances which may be electrolytically dissociated into sulphur vapor and pure elements, thus producing the constituents by a single continuous automatic process.

It is a further object of this invention to provide a method of mining including the displacement of minerals by a circulating medium which may, itself, be later removed by displacement with a cheaper medium.

One other object is to provide a continuous process of mining and refining the minerals mined.

Other objects and advantages of this invention will become apparent from the following description taken in connection with the accompanying drawings, it being understood that same are by way of illustration only, and not by way of limitation.

5

10

15

20

25

30

35

40

45

50

55

Fig. 1 is a diagrammatic illustration of an apparatus which may be used in the carrying out of a process of mining in accordance with this invention.

5 Fig. 2 is a vertical cross section of the lower portion of a well illustrating diagrammatically a slightly modified well arrangement for use in connection with this invention.

10 Fig. 3 illustrates still another form of well arrangement.

Fig. 4 illustrates a fourth form of arrangement of wells for use in connection with this invention.

In practicing the present invention there is employed a circulating medium consisting for 15 example of molten or superheated sulphur or a medium containing sulphur or having certain of its attributes.

For the removal of minerals from the ground, Fig. 1 illustrates a set-up in which two wells 20 have been drilled to spaced points in the ore stratum. These wells may be drilled in any acceptable manner, the details thereof forming no part of this invention. They are designated in Fig. 1 of the drawings by the numerals 1 and 25 2, respectively. After the two wells have been drilled, a channel is opened along the mineralized fractures between the wells by some means such as for example the detonations of an explosive charge at the bottom of one or both 30 wells within the producing formation. If detonations are caused in both wells, they may be simultaneous or spaced as to time. These detonations may be repeated of course as many 35 times as may be necessary to open up a channel between the wells.

To the well designated by the numeral 2, which may be termed the outlet well, is connected a pipe 3 leading to the lower end of a gravity separator chamber 4 having a gas outlet 40 5 at its upper end. Leading from a point intermediate the ends of the separator 4 in a substantially horizontal direction is a pipe 6 extending over a trap 7 and this pipe and an exhaust pipe 8 leading from the lower end of the 45 separator, are connected to a concentrator chamber 9. Leading from spaced points along the height of the concentrator 9 are lead-off pipes numbered 11, 12, 13, 14 and 15, respectively, the highest being numbered 11, and the 50 lowest 15. A vapor conduit 16 leads from the upper end of the concentrator to the intake of the compressor 17, the outlet 18 of which leads to a boiler 19.

The lead-off pipes 11 to 15 lead respectively 55 to the interiors of a bank of electrolytic cells. Each of these cells has a shell 20 containing a floating anode 21 of carbon or the like, the shell 20 providing the cathode. The shell 20 is thus connected by a conductor 22 to the negative pole 60 of a source of electrical energy, and the anode 21 by a conductor 23 to the positive pole of such source. The carbon anode 21 is provided with vertical openings therethrough to increase the surface of contact with the electrolyte and permit 65 the ready escape of gas given off during use of the cell. It is also provided with an opening which extends only part-way therethrough from the bottom toward the top and is adapted to cooperate with an insulated guide post extending 70 up from the bottom of the shell 20 to prevent the anode from contacting the inner walls of the shell 20 and short-circuiting the cell. The last mentioned opening serves also to trap a quantity of gas and assist in keeping the anode 75 afloat in the electrolyte.

Leading off from the upper end of each shell 20 is a vapor pipe 24 which is joined to the line 16 at 25 before the pipe 16 enters the compressor 17. From the lower end of this shell 20 extends a drain pipe 26. Leading from the 5 dome of the boiler 19 is a pipe 27 which connects the boiler to the well 1 which may be termed the input well. It is to be understood that additional pumping facilities may be provided if necessary to maintain circulation. A 10 second pipe 28 leads from the boiler dome to the extreme lower end of the concentrator 9 as shown at 28a, and has a branch 28b which leads to the lower end of a reducing tower 29 having a body or bodies of carbon disposed therein and 15 shown at 29a.

A compressor 30 is connected to the opening 5 at the upper end of the separator 5 and the discharge thereof is connected likewise to the lower end of the reducing tower 29. Adjacent 20 the upper end of the reducing tower 29 is a pipe 31a leading from the reducing tower through a pressure reduction valve 31b to the top of the concentrator, and at the extreme upper end of the reducing tower 29 there is provided a pop- 25 off or relief valve 31c.

After the channel between the two wells has been opened as above set forth, any suitable heated circulating medium may be forced down through one well and up through the other until 30 the system has become heated to such an extent that molten sulphur may be introduced and circulated without substantial loss of heat. The molten sulphur having been heated in the boiler 19 is then forced into one of the wells under 35 pressure and circulated through the two wells by means of the compressor 17 displacing the previously circulated liquid medium. In passing through the producing stratum between the two wells, the molten sulphur will be brought 40 into intimate contact with the ores containing the minerals to be removed.

Thermochemical mining of minerals from their ores consists of altering them by means of a molten displacement medium which will produce 45 them in suspension or solution when it is circulated through the ore body and vaporized at the surface in order to obtain the concentrated altered minerals.

In the case of molten sulphur circulated 50 through a body containing cupric oxide in an enclosed system, the oxide is immediately attacked by the sulphur, forming cupric sulphide and sulphur dioxide which are both dissolved by the molten sulphur.

It is also worthy of note that in the practice of this method whenever the molten sulphur comes in contact with water during circulation through the ore body the water is attacked immediately by the sulphur forming hydrogen 60 sulphide and sulphur dioxide, both of which are appreciably dissolved in the sulphur. The hydrogen sulphide thus formed is characteristic of this system of mining because when molten sulphur is forced into a well as in carrying out the present process, the molten sulphur medium will contact water of hydration and crystallization, as well as certain other moisture which may be artificially introduced at the surface. The hydrogen sulphide formed as just 70 set forth will at least partially dissolve in the molten sulphur and supply sulphide ions which in turn will be consumed by the chemical alteration of the native minerals to sulphides.

The hydrogen sulphide production either in

the above examples or in this mining method is limited by the enclosed system to that which will dissolve in the molten sulphur at the existing pressures and temperatures. Consequently, although the concentration of the hydrogen sulphide ions is relatively small, the speed of their replenishment will depend upon the speed at which they are consumed by the alteration of such minerals as native copper to cupric sulphide.

10 The alteration of these minerals will thus be stimulated in some cases by the presence and consumption of the sulphide ions supplied by the dissolved hydrogen sulphide. The alteration of other minerals, such as the metallic oxides, will 15 not be stimulated by the presence of these sulphide ions, but will be the result of the direct replacement of oxygen by sulphur, or of some other constituent of the mineral by sulphur.

The concentration of the dissolved sulphur dioxide will thus depend on the amount of mineral alteration and consequently will be large. Since the equilibrium between the hydrogen sulphide and sulphur dioxide formed from water and sulphur must be maintained, excessive quantities of sulphur dioxide will inhibit the formation 25 of hydrogen sulphide unless it is removed from the system. This may be accomplished most readily at the separator 4 where the escape of all gases from the system is permitted, as herein-after described.

The minerals found in the earth are generally classified according to the chemical activity of the metals they contain. Those which are comparatively inactive occur generally as free or 30 native metals or as sulphides. Those which are comparatively active occur generally in very stable forms such as silicates, titanates, tantalates and fluorides, and the intermediate group occur ordinarily as oxides, carbonates, sulphates and 35 sulphites.

Of this inactive group, those occurring as sulphides are for the most part soluble in sulphur, while those which occur as native elements may be divided into two classes. The first of these 40 classes consists of those which fall into groups IB, IIB, IVA and VA of the periodic table, since these have an affinity for sulphur, and hence will combine with molten sulphur to form sulphides and may then be carried off either in solution or 45 in suspension. This class of native elements is particularly reactive with sulphide ions, as supplied by dissolved hydrogen sulphide. The second of these classes, consisting of those falling in the remaining groups of the periodic table, 50 show relatively slight affinity for molten sulphur and hence will not to any substantial degree combine with sulphur and consequently cannot be removed by this method.

The active or highly oxidized group, such as 55 the silicates, will, in most instances, not react with molten sulphur, but may, in some instances, react with sulphur to form thionates. That is, some of the oxygen atoms will be replaced by sulphur atoms. The solubility of such thionates in sulphur is appreciable.

The intermediate group may be similarly produced by the present medium in solution and suspension, the oxides being altered to sulphides 60 by the direct replacement of the oxygen atoms by sulphur atoms and by the consequent formation of sulphur dioxide and the mineral sulphide. The carbonates will ordinarily remain inert and will not dissolve or be otherwise altered. The sulphates and sulphites are in general effectively

soluble in the molten sulphur, and will thus be produced in solution or suspension.

From the foregoing, it will be noted that strictly speaking the removal of the minerals by means of circulating a sulphurized medium, such as above contemplated, is not a removal by displacement, but is instead a removal by alteration and conduction. That is to say, while the removed ores are of course replaced by the sulphur medium, they are not removed by displacement. Instead, there is the chemical alteration 10 and the subsequent conduction or carrying off of the products of this alteration by the highly heated circulating medium which provides for the removal of the minerals and not simply their 15 displacement by the circulating medium.

When the mineral-laden molten sulphur arrives at the top of the second well, it is then conducted through a series of treatments which may be independent of the nature of the mineral 20 which is being removed. The sulphuretted mineral as above pointed out will be found in the circulating medium generally in the form of a sulphide either in solution or in suspension, and the circulating medium will also be found to contain considerable quantities of sulphur dioxide produced by the reaction of the molten sulphur with minerals and moisture during the process.

When this circulating medium carrying the minerals and various gases arrives at the top of 30 the well, therefore, it will be found necessary to put it through a number of separation steps which, by way of example, may be as follows:

First, the circulating medium is led through the line 3 from the well 2 to the separator 4 where 35 by gravity the light, inert substances suspended in the sulphur, such as the siliceous impurities of the gangue, etc., will be separated. In this device, any steam which may exist, as well as the sulphur dioxide and other gases, will be permitted to escape through the upper end of the separator, and any floatable impurities will be caused to pass off through the line 6 and out through the trap 8. The stream conveying such floating impurities to the trap 7 will pass on and 40 into the concentrator 9. The sulphurized medium still containing the mineral constituents from the ground will be conducted by means of the line 8 into the bottom of the concentrator 9 where 45 in the sulphurized medium will be vaporized, and the disseminated sulphides produced by displacement of the activated minerals will be separated by differential floating in the rising medium within the concentrator or vaporizer 9.

The altered minerals, depending upon whether 50 they are light sulphides or heavy sulphides, will be removed through the lines 11, 12, 13, 14 and 15. The sulphur vapor will pass off through the vapor line 16 to the intake end of the compressor 17 where it will be reliquified and conducted 55 through the line 18 to be injected into the boiler 19. It is noted that the gases passing off from the upper end of the separator are compressed by the compressor 30 and forced through the reducing tower 29 containing the carbon 29a. The 60 concentrator 9 and the reducing tower 29 are heated by means of super-heated sulphur conveyed through the lines 28, 28a and 28b from the boiler 19. In the reducing tower the sulphur in the sulphur dioxide is replaced by carbon so as 65 to form carbon dioxide and free liquid sulphur. The carbon dioxide then escapes through the valve 31c, whereas the liquid sulphur will pass off through the line 31a through the pressure reduction valve 31b, and into the upper end of the 70 75

concentrator 9 where in vapor form it will be carried off through the line 16 to the compressor 17. Any steam discharged from the relief valve 5 will also be discharged from the relief valve 31c, unless altered to sulphur dioxide and hydrogen sulphide in the reducing tower 29, such sulphur dioxide being reduced to liquid sulphur and carbon dioxide, as above.

The hot sulphides from the concentrator 9, which sulphides pass out through the lines 11, 12, 13, 14 and 15, are conducted to the series of electrolytic cells where they will be dissociated into the liquid metals and boiling sulphur. The sulphur vapor from these electrolytic cells is carried off through the lines 24 from the tops of the respective cells, which lines join at 25 the sulphur vapor line 16 so that all the sulphur vapor is conducted to the compressor 17 as previously set forth. Each of the cells adjacent its lower portion is provided with a discharge line 26 through which the liquid metals will be discharged from the electrolytic cells.

The heat losses from the concentrator 9 are not necessarily large, even though the sulphur medium is being removed by vaporization at the top of this unit, since the pressure maintained in the concentrator is less than one atmosphere as a result of the suction created by the compressor, thus lowering the vaporization temperature below the normal boiling point of the sulphur. The temperature of the electrolytic cells on the other hand is relatively high in order that the dissociated metals may be continuously removed as liquids from the electrolytic cells where in they have acted as liquid cathodes. The vertical separation of the cathodes from the anodes in these cells may be controlled by the rate at which the metals are removed from the cells.

The boiler 19 which provides the superheated sulphur which is used in this circulation process is connected by means of a line 27 to the well 1 so that sulphur from the boiler will pass back again through the well 1 and into the formation to repeat the cycle.

While it is desirable in many instances where it may be possible to have the circulation take place as above described, employing two wells and circulating the fluid along a path between the two wells through the producing formation, it is conceivable that a formation might be encountered of such a nature and in such a location as to make this impractical. In such instances, it is contemplated that a single well may be employed such as illustrated at 32 in Fig. 2, and the circulation of the sulphurized medium in that instance would be caused to take place downwardly through a tubing 33 at the bottom of which it would be directed laterally by means of nozzles 34 or the like, to wash against the walls 35 of the cavity in the formation at the bottom of the well. The surface casing 36 extends downwardly to the upper end of the cavity and is open at its lower end as indicated at 37. Thus, a hot circulating fluid passed downwardly through the tubing would be propelled with considerable velocity through the nozzle-like openings 34 and caused to wash against the walls 35 of the producing formation. The ores contained in the formation would be transformed in the same manner as in the previously described process, and the

sulphur carrying the minerals would then be passed upwardly through the lower end 37 of the surface casing and up through the casing into the separating apparatus previously referred to.

Another arrangement desirable in instances where the producing formation is at a steep inclination is shown in Fig. 3. In this case, the well 38 is drilled so as to extend into and along the producing stratum. The tubing 39 is then placed in the cased well and the heated sulphur forced down the tubing and up around the tubing, thus contacting the ore body along a considerable distance as it returns around the tubing. As in Fig. 2, the tubing may be raised or lowered as the formation becomes exhausted, but to a greater extent in this instance because the well extends along the stratum instead of through it transversely.

In Fig. 4 the well is drilled along the stratum as in Fig. 3, but a second well 41 is provided for the return or output well, and the circulation takes place in a manner similar to that described in connection with Fig. 1.

In all the various arrangements shown the chemical reactions will be the same, and the same apparatus and process may be employed in separating the minerals from the circulating medium.

It will be appreciated from the foregoing that there may be many immaterial variations of the process set forth without departing from the spirit or scope of this invention.

It is intended that the scope of this invention shall cover all such variations as may fall within the terms of the appended claims.

Having described my invention, I claim:

1. In a method of mining, the steps of circulating molten sulphur through an ore deposit, and treating the molten sulphur as it comes from said ore deposit to remove therefrom minerals taken up by the molten sulphur from the ore deposit.

2. In a method of mining, the steps of circulating a molten sulphur through an ore deposit, permitting the gas contained in said molten sulphur to escape therefrom as it comes from the ore deposit, vaporizing a portion of said molten sulphur, and performing electrolysis on the remainder of said molten sulphur to separate therefrom the mineral constituents taken up from said ore deposit.

3. In a method of mining, the steps of circulating a molten sulphur through an ore deposit, permitting the gas contained in said molten sulphur to escape therefrom as it comes from the ore deposit, vaporizing a portion of said molten sulphur, performing electrolysis on the remainder of said molten sulphur to separate therefrom the minerals taken up from said ore deposit, recovering sulphur from the gases given off by said molten sulphur, and re-liquifying the vaporizing sulphur, reheating the total recovered sulphur and re-circulating the same.

4. In a method of mining, the steps of circulating sulphur through an ore deposit, and treating the sulphur as it comes from said ore deposit to remove therefrom minerals taken up by the sulphur from the ore deposit.